

Patented Sept. 27, 1927.

1,643,355

# UNITED STATES PATENT OFFICE.

GEORGE A. RICHTER AND MILTON O. SCHUR, OF BERLIN, NEW HAMPSHIRE, AS-  
SIGNORS TO BROWN COMPANY, OF BERLIN, NEW HAMPSHIRE, A CORPORATION OF  
MAINE.

## PROCESS FOR THE MANUFACTURE OF HIGH ALPHA-CELLULOSE FIBER.

No Drawing. Application filed April 9, 1925, Serial No. 21,963. Renewed November 3, 1926.

This invention relates to the preparation of high alpha-cellulose fiber. High alpha-cellulose fiber may be produced by cooking unbleached sulphite pulp with an alkaline 5 cooking liquor (a caustic soda solution being especially adapted for this purpose), and then bleaching the cooked product. This cooking may take place at any suitable temperature and pressure, although we have 10 found it to be more economical and expedient to cook in open tanks under atmospheric pressure. The alkali in solution reacts with and dissolves the lignin and the less resistant beta and gamma celluloses present in the 15 pulp, so that when the liquor is drawn off after the necessary period of digestion the resultant product is easy to bleach and contains at least 94% alpha-cellulose fiber. High alpha-cellulose fiber may be employed 20 as a substitute for cotton fiber in paper making and in the preparation of the cellulose esters, the cellulose ethers, and in the preparation of other compounds which require the use of substantially pure cellulose. 25 A drawback to the use of caustic soda alone as the alkaline digesting agent is, however, that it renders the process expensive.

The object of this invention is to provide 30 a more economical method for the preparation of a high alpha-cellulose fiber, yielding a product which will possess the same characteristics as that produced by the use of caustic soda. Briefly, this is attained by cooking the pulp in slaked lime cooking 35 liquor and in caustic soda liquor. Other advantages which may be obtained in this invention will subsequently be pointed out.

In a co-pending companion application 40 filed of even date herewith, Serial No. 21,962, which has become Patent No. 1,599,489, the use of milk of lime has been described as being effective in removing beta and gamma cellulose from unbleached sulphite pulp but it is pointed out that the caustic soda cooking 45 liquor is much more effective in removing the coloring matters therefrom. In order to produce fiber of high whiteness, these coloring substances must be removed. In that 50 application we have pointed out that in order to sufficiently whiten the pulp after an ordinary lime-digestion, it is necessary to use an excess of bleach, thereby resulting in a weakening of the fiber and a reduction of the alpha-cellulose content.

We have found that unbleached sulphite 55 pulp may be cooked with a mixture of slaked lime ( $Ca(OH)_2$ ) and caustic soda ( $NaOH$ ), the proportions of these re-agents and the method of using them being so chosen that the beta and gamma celluloses and the lignin 60 and other coloring matter are dissolved and thereby removed therefrom. The cooked product upon mild bleaching is very white and contains over 94% alpha cellulose.

While a mixed caustic and lime cooking 65 liquor may be employed, the pulp may be cooked first in caustic soda liquor and the lime added later thereto, or it may be cooked in a lime liquor first and the caustic added later,—the last procedure being preferred, 70 for in this case the lime reacts with the less resistant beta and gamma celluloses first, and the caustic soda added later is consumed substantially only in the removal of the lignin and other coloring matter. If it were 75 added otherwise it might also be consumed in reacting with the less resistant celluloses rather than with the coloring substances. Although a gain in bleachability of the product 80 may be secured by washing the stock between the alkaline treatments, for reasons of economy in steam and equipment it is preferred to add the latter alkali directly 85 after the first alkali treatment has been completed. The method may be practiced about 85 as follows:—

A 10% suspension of unbleached sulphite pulp is mixed thoroughly with milk of lime containing about 6% to 8% active calcium oxide based upon the bone-dry fiber weight. 90 The mixture is brought to about  $200^{\circ}$  to  $210^{\circ}$  F. in an open tank by means of live steam, and is thoroughly agitated while being maintained at this temperature for from five to eight hours, depending upon the characteristics of the particular sulphite stock undergoing treatment. The beta and gamma celluloses react with and are effectively removed by the lime. Then 1% to 2% caustic soda based upon the bone-dry fiber is 95 added preferably in the form of a boiling-hot 1% to 5% solution, and is thoroughly mixed with the pulp. About an hour after the addition of the caustic soda, the lignin and other coloring matters have reacted sufficiently therewith, and the stock is then washed clear of reaction products. From 100 4% to 6% of bleach ( $CaOCl_2$ ), based on the 105

weight of dry fiber, in the subsequent bleaching operation gives a very white alpha-cellulose fiber having the characteristics required.

5 The stock leaving the cooking-tanks has approximately the following characteristics:—Alpha-cellulose 94%, fiber length 0.9–1.1 mm., copper number 1.4–2.0.

10 After the bleaching, the characteristics are substantially the same, with the exception of the color; the whiteness is 95 to 100 on our scale, and may be increased without injury to the fiber to 100 to 110 by a superbleaching process, in which the pulp is treated with a 15 chlorine solution.

15 It may be advantageous to combine a chlorine solution pre-treatment which removes or renders reactive a portion of the lignin in the sulphite pulp prior to the practice of 20 the previously described process, so that economy in the use of chemicals may further be increased with the easier attainment of a very white alpha-cellulose product. This may be done by treating the unbleached sulphite pulp prior to the alkaline digestion 25 with a chlorine solution, a portion of the lignin and other coloring substances reacting with and being oxidized by the chlorine. Such a pre-treatment would make possible 30 the use of less caustic in the subsequent alkaline cook.

35 Another important advantage may be obtained by the use of the chlorine pre-treatment process, which is that the wood chips 40 may be slightly undercooked in the sulphite digesters, thus producing a longer fiber. The pulp thus obtained would ordinarily be more difficult to bleach owing to the fact that it contains a higher percent of lignin, 45 but the quantity of oxidizing agents used in the pre-treatment may be increased so as to remove or render more reactive the additional amount of lignin. The pre-treated pulp will then be subjected to the caustic and 50 lime cooking solution and upon bleaching will yield a very white alpha-cellulose fiber of the desired chemical and physical characteristics.

55 It is, of course, possible to replace all or a part of the caustic soda by other strongly alkaline substances which readily react with the lignin and other coloring substances in the unbleached sulphite pulp, such, for example, as sodium sulphide ( $Na_2S$ ) or sodium polysulphide ( $Na_2S_x$ ) or caustic potash (KOH); and dolomite lime, containing magnesium oxide, may be used in place of all or part of the calcite lime. Furthermore, it is not necessary that the processes be carried 60 out in open tanks. Closed digesters may be used and the alkaline treatment carried out under higher temperature and pressure conditions, in which case the caustic solution in the foregoing example would be introduced 65 into the digester by a pump, injector, or

other suitable means. It is to be emphasized, on the other hand, as in the copending application, Serial No. 21,962, which has become Patent No. 1,599,489, that the use of high temperature and pressure would complicate the process and call for the use of a comparatively intricate apparatus, all of which tends to make the process as or more expensive than a straight caustic soda treatment.

70 Since lime is much cheaper than an equivalent quantity of caustic soda and is effective in removing the beta and gamma celluloses from the pulp, the foregoing process is more economical than a straight caustic soda treatment in proportion to the percentage of lime which may be substituted for caustic. We do not herein claim broadly a process of 75 initially treating a sulphite pulp with an oxidizing agent, then digesting the pulp with an alkaline reagent under heat and at atmospheric pressure, and finally bleaching the product, as this forms the subject-matter 80 of our application Serial No. 716,154, filed 85 May 27, 1924.

90 What we claim is:

1. The process of producing a high alpha-cellulose fiber, which comprises cooking unbleached sulphite pulp in a solution of an alkaline compound of an alkali metal, containing in suspension an alkaline earth metal hydroxide.

95 2. The process of producing a high alpha-cellulose fiber, which comprises cooking unbleached sulphite pulp in a suspension of an alkaline earth metal hydroxide, adding a solution of an alkaline compound of an alkali metal, and continuing the cooking.

100 3. The process of producing a high alpha-cellulose fiber, which comprises cooking unbleached sulphite pulp at atmospheric pressure in a suspension of lime, adding a solution of sodium hydroxide, and continuing the cooking.

105 4. The process of producing a high alpha-cellulose fiber, which comprises treating unbleached sulphite pulp with a solution of chlorine, insufficient in quantity to cause complete bleaching, boiling with a suspension of lime, adding a solution of sodium hydroxide and continuing the boiling.

110 5. The process of producing a high alpha-cellulose fiber, which comprises treating unbleached sulphite pulp with a solution of chlorine, insufficient in quantity to cause 115 complete bleaching, separating the pulp from soluble reaction-products, boiling it with a suspension of lime, adding a solution of sodium hydroxide, continuing the boiling, and again separating the pulp from soluble 120 reaction products.

125 6. The process of producing a bleached high alpha-cellulose fiber, which comprises cooking unbleached sulphite pulp with a suspension of lime, adding a solution of sodium

hydroxide, continuing the cooking, separating the pulp from soluble reaction-products, and bleaching it with calcium hypochlorite solution.

5 7. The process of producing a super-bleached high alpha-cellulose fiber which comprises cooking unbleached sulphite pulp with a suspension of lime, adding a solution of sodium hydroxide, continuing the cooking, separating the pulp from soluble reaction products, bleaching it with calcium hypochlorite solution and superbleaching it with a chlorine solution.

10 8. The process of producing a high alpha-cellulose pulp, which comprises cooking unbleached sulphite pulp in a lime suspension containing about 6% to 8% calcium oxide based on the weight of bone-dry fiber and in a caustic soda solution containing 1% to

2% sodium hydroxide based on the weight <sup>20</sup> of bone-dry fiber.

9. The process of producing a high alpha-cellulose pulp, which comprises undercooking chips in a sulphite digesting liquor, treating the product obtained from said sulphite digesters with chlorine to eliminate a portion of the lignin but without causing a complete bleaching reaction, and cooking said treated product with agitation in a milk of lime suspension to remove beta and gamma celluloses therefrom, adding a caustic soda solution to the mass and continuing the cooking to remove more ligneous matter therefrom.

15 In testimony whereof we have affixed our <sup>31</sup> signatures.

GEORGE A. RICHTER.  
MILTON O. SCHUR.